

(No Model.)

E. POPPONITSCH.  
PRIMARY ELECTRIC BATTERY.

No. 511,159.

Patented Dec. 19, 1893.

Fig: 1



Fig: 2



Fig: 3.



WITNESSES:

Charles Kable  
Harry Willard Griffiths

INVENTOR

*Edward Poppowitzch*  
BY  
*Joseph Baeguer*  
ATTORNEYS.

# UNITED STATES PATENT OFFICE.

EDWARD POPPOWITSCH, OF BROOKLYN, ASSIGNOR OF ONE-HALF TO  
HERMAN WÜSTENFELD, OF NEW YORK, N. Y.

## PRIMARY ELECTRIC BATTERY.

SPECIFICATION forming part of Letters Patent No. 511,159, dated December 19, 1893.

Application filed December 28, 1892. Serial No. 456,588. (No model.)

*To all whom it may concern:*

Be it known that I, EDWARD POPPOWITSCH, a subject of the Emperor of Austria-Hungary, residing at Brooklyn, in the county of Kings 5 and State of New York, have invented certain new and useful Improvements in Primary Electric Batteries, of which the following is a specification.

This invention relates to that class of open 10 circuit galvanic batteries known as "dry batteries," and the object of my invention is to produce a simple, cheap and very effective battery, in which the zinc can be readily replaced by new ones after they are spent, and 15 in which a constant current of high electro-motive force is obtained until the zincs are entirely used up.

The invention consists of a galvanic-battery comprising an acid-proof containing jar, 20 carbon-plates and zincs supported therein from the top of the jar, and a packing within the space around the carbons and zincs consisting of sawdust, sea-salt, sal-ammoniac, granulated manganese and concentrated sul- 25 phuric-acid, which packing is moistened from time to time by supplying a small quantity of water through a plugged opening in the top of the containing-jar, thereby forming a wet packing embedding the positive and neg- 30 ative plates.

In the accompanying drawings, Figure 1 represents a vertical transverse section of my improved galvanic battery, on line 1 1, Fig. 3. Fig. 2 is also a vertical transverse section of 35 the same taken at right-angles to the plane of Fig. 1, on the line 2 2, Fig. 3, and Fig. 3 is a plan-view of the battery.

Similar letters of reference indicate corresponding parts.

40 In the drawings, A represents a containing-jar which is constructed of sheet-metal and coated at the interior and exterior surfaces with a layer of asphaltum or other acid-proof material. The top-plate A' of the jar A is made of the same material and supports the carbon-plates C C which are inserted into 45 openings in the top-plate, said carbons being provided with binding posts at their upper projecting ends for the conducting wires. 50 The top-plate A' is provided at two or more

points with openings and fixed downwardly-extending sleeves a through which the zincs B B are inserted, the upper ends of the zincs projecting like the upper ends of the carbons above the top-plate of the jar and being provided with binding screws for the conducting wires. The spaces between the carbon-plates, zincs and the wall of the containing-jar is packed tightly with sawdust that is mixed with an exciting solution composed of ten 60 parts of sea-salt, ten parts of sal-ammoniac, ten parts of bi-chromate of potash, ten parts of mercury, ten parts of granulated manganese and one part of concentrated sulphuric acid. All these ingredients are mixed with 65 the sawdust in dry state, the sulphuric acid being added last, thus forming a packing all round the zinc and carbon-plates, so that the full benefit of the excitants may be obtained.

To start the battery, the packing is supplied with a small quantity of water, which is inserted through an opening in the top-plate, which opening is closed by a suitable plug d, after the water is supplied. From time to time the jar is supplied with a new 70 quantity of water. This is continued from time to time until the zincs are entirely used up. The zincs can then be readily replaced by new ones when they are used up. This is readily accomplished by withdrawing the old 75 zincs from the sleeves of the top-plate and inserting new ones into the same. The zincs can also be removed from time to time, cleaned and re-inserted, the battery retaining its moisture for a long time and furnishing 80 a constant current of high electro-motive force. By re-supplying a small quantity of water from time to time, the life of the battery can be extended for a considerable length of time.

Having thus described my invention, what I claim as new, and desire to secure by Letters Patent, is—

1. An electric-battery, composed of a closed acid-proof containing-jar, positive and negative plates supported in said jar, and a packing of sawdust, sea-salt, sal-ammoniac, bi-chromate of potash, granulated manganese and concentrated sulphuric-acid, mixed in or about the proportions specified.

2. In an electric-battery, a packing for separating the positive and negative plates, composed of a mixture of saw-dust, sea-salt, sal-ammoniac, bi-chromate of potash, mercury, 5 granulated manganese and concentrated sulphuric acid, substantially as set forth.

In testimony that I claim the foregoing as

my invention I have signed my name in presence of two subscribing witnesses.

EDWARD POPPOWITSCH.

Witnesses:

PAUL GOEPEL,

HARRY WILLARD GRIFFITHS.